

1

3,245,905

BLENDED FIBERS HAVING IMPROVED  
ANTISTATIC PROPERTIES

Charles C. White and Raymond E. Donaldson, Kingsport, Tenn., assignors to Eastman Kodak Company, Rochester, N.Y., a corporation of New Jersey  
No Drawing. Filed Oct. 9, 1962, Ser. No. 229,486  
5 Claims. (Cl. 252—875)

This invention relates to novel compositions of matter for use in the textile art. More particularly, this invention relates to novel antistatic and lubricating compositions for treating textile fibers and to fibers treated therewith.

Lubricants and like compounds are usually applied to textile fibers, filaments, yarns and the like to reduce the tendency toward breakage of the individual filaments when they are subjected to various mechanical strains, and to lubricate the individual filaments in order to facilitate handling in such operations as spinning, twisting, winding, reeling, drafting, weaving, carding, combing, and the like.

Textile fibers also tend to accumulate electrostatic charges during the various handling operations such as spinning, twisting, winding, and the like. The accumulation of electrostatic charges causes the fibers to become electrically repellent to one another and to become electrically attracted to the equipment on which they are handled. As is known in the art, such a condition is highly undesirable in that it interferes substantially with the efficiency and effectiveness of processing operations. It is therefore desirable that the applied composition reduce substantially or completely eliminate the tendency of the treated textile fibers to accumulate undesirable electrostatic charges during processing.

The new synthetic resin fibers such as those prepared from polyester resins, polyamide resins, polyolefin resins, and resins prepared by the polymerization and copolymerization of certain acrylic compounds have proved highly satisfactory for use in the textile industry. These fibers, which normally have hydrophobic properties, are used in the manufacture of fabrics and like materials. Often, these hydrophobic fibers are blended or associated with hydrophilic fibers such as cotton, wool, viscose and the like to provide fabrics having certain desired properties.

Various lubricating and antistatic compositions have been proposed for treatment of the above-mentioned hydrophobic synthetic resin fibers. However, these compositions have not proved entirely satisfactory in use.

One particular problem involved in the use of known treating compositions is that, when hydrophobic fibers treated therewith are blended with hydrophilic fibers, the applied composition tends to migrate to the hydrophilic fibers leaving the hydrophobic fibers substantially devoid of antistatic protection and satisfactory frictional characteristics.

This invention has for one of its objects novel antistatic and lubricating compositions for application to hydrophobic fibers.

Another object of this invention is a textile fiber treated with the novel antistatic and lubricating compositions of this invention.

Other objects of this invention will, in part, be obvious and will, in part, appear hereinafter.

For a complete understanding of the nature and the objects of this invention, reference is made to the following detailed description.

Briefly, in accordance with this invention, there are provided novel antistatic and lubricating compositions adapted particularly to be applied to textile fibers having hydrophobic properties such as textile fibers prepared

2

with polyamide resins, polyester resins, polyolefin resins, acrylic resins, and the like whereby there is provided treated textile fibers having outstanding antistatic properties and frictional properties.

The base antistatic and lubricating composition of this invention is comprised of, by weight, (A) from about 20 parts to 75 parts of a water-soluble compound which is a mixture of monohydroxy oxyethylene oxy 1,2-propylene aliphatic monoethers having a viscosity of from about 200 to 700 Saybolt Universal Seconds at 100° F. and in which ethylene oxide and 1,2-propylene oxide are combined therein as oxyethylene and oxy 1,2-propylene groups in a weight ratio of 1,2-propylene oxide to ethylene oxide of from 60:40 to 40:60, the monoethers of said mixture containing in a single molecule both the oxyethylene group and the oxy 1,2-propylene group, (B) from about 5 parts to 35 parts of lauryl acid phosphate, (C) from about 1 part to 10 parts of morpholine, (D) from about 5 parts to 25 parts of polyoxyethylene glycol having a molecular weight of from about 1,000 to 2,000, and (E) from about 1 part to 5 parts of o-phenylphenol.

While the above composition has proved highly satisfactory in use, other components can be incorporated therein, if desired, to improve to some degree the antistatic and/or lubricating properties thereof.

Thus, while the antistatic properties of the above base composition are highly satisfactory for most applications, the antistatic properties can be improved somewhat by the incorporation therein of from about 5% to 30% by weight, based on the total weight of the base composition, of polyoxyethylene lauryl amine wherein the polyoxyethylene group has an average molecular weight of about 200. This compound can be prepared by reacting lauryl amine with ethylene oxide, the ethylene oxide being employed in an amount sufficient to provide a polyethylene lauryl amine wherein the polyoxyethylene group has an average molecular weight of about 200. Such a compound is available commercially as Atlas G 3780A.

Also, the antistatic properties can be improved by the addition to the base composition of the N,N-diethylaminoethanol salt of oleyl sulfate. The amount employed will be from about 5% to 25% by weight, based on the total weight of the base composition. This compound has the structural formula



Component (A) of the base composition is a mixture having relatively high molecular weight and which comprises molecules containing polyoxyalkylene chains formed predominantly of the oxyethylene group  $-\text{OC}_2\text{H}_4-$ , and the oxy 1,2-propylene group,



Such mixture can result, for instance, from the reaction of a monohydroxy aliphatic alcohol such, for example, as butanol with alkylene oxide mixtures containing, for the most part, ethylene oxide and 1,2-propylene oxide.

60 A mixture of monohydroxy oxyethylene oxy 1,2-propylene aliphatic monoethers can be prepared by adding a substantially aldehyde-free mixture of ethylene oxide and 1,2-propylene oxide to an aliphatic monohydroxy alcohol having from about 1 to 10 carbon atoms such, for example, as butanol, under substantially anhydrous conditions in an amount which is at least about 6 moles of said oxides for each mol of alcohol, the oxides present in said mixture being comprised of, by weight, from about 60 to 40 parts of 1,2-propylene oxide and from about 40 to 60 parts of ethylene oxide. The preferred mixture of oxides is about equal parts, by weight, of the

oxides. That is, in the oxide mixture, there is present for each one part by weight of ethylene oxide, one part by weight of 1,2-propylene oxide.

The mixture of oxides is added at such rate as to maintain a substantially uniform concentration of unreacted oxide in the reaction zone while maintaining the reaction mixture at a temperature of from about 80° C. to 160° C. and at a pressure of from about 5 p.s.i. to 50 p.s.i.

Mixtures of monohydroxy oxyethylene oxy 1,2-propylene aliphatic monoethers and their method of preparation are disclosed and described in Patent 2,425,755 of August 19, 1947, reference to which is hereby made. Mixtures of monohydroxy oxyethylene oxy 1,2-propylene aliphatic monoethers are available commercially under the proprietary designation Ucon. As set forth hereinabove the preferred mixture of monohydroxy oxyethylene oxy 1,2-propylene aliphatic monoethers are those which have a viscosity of from about 200 to 700 SUS (Saybolt Universal Seconds) at 100° F.

#### Example I

Particularly suitable as component (A) is a mixture of monohydroxy oxyethylene oxy 1,2-propylene butyl monoethers having a viscosity of about 300 SUS at 100° F. and in which ethylene oxide and 1,2-propylene oxide are combined therein as oxyethylene and oxy 1,2-propylene groups in a ratio which is about one part of 1,2-propylene oxide for each part of ethylene oxide, by weight, the monoethers of said mixture containing in a single molecule both the oxyethylene group and the oxy 1,2-propylene group. This mixture is prepared as hereinbefore described using butanol as the aliphatic monohydroxy alcohol. Such a mixture is available commercially under the proprietary designation Ucon 50 HB 260.

The lauryl acid phosphate component (B) can be either dilauryl phosphate ( $C_{12}H_{25}$ )<sub>2</sub>HPO<sub>4</sub>, monolauryl phosphate ( $C_{12}H_{25}$ )H<sub>2</sub>PO<sub>4</sub>, or mixtures thereof.

The polyoxyethylene glycol component (D), also referred to in the art as polyethylene glycol, employed in preparing the base composition of this invention can be polyoxyethylene glycol having an average molecular weight of from about 1,000 to 2,000. These compounds are well known in the art and are available commercially. Thus, for example, a polyoxyethylene glycol having an average molecular weight of about 1540 is available commercially under the proprietary designation Carbowax 1540.

In preparing the novel lubricating and antistatic compositions of this invention, the components in the desired amounts are admixed or blended together in any conventional manner such, for example, as by blending in a high-speed blender or by stirring with a motor-driven stirrer.

The base compositions of this invention are either completely soluble or completely dispersible in water depending on the water solubility of the individual components of which the formulation is comprised. Thus, the application of the novel composition of this invention to textile fibers is conveniently and preferably accomplished by employing water as a vehicle or carrier therefor. The aqueous solution or dispersion can be applied to textile fibers in any conventional manner such, for example, as by immersion, by wick application, by roll application, or by spraying.

The aqueous solutions or suspensions of the compositions of this invention will usually comprise from about 5 parts to 25 parts by weight of the composition and from about 95 to 75 parts by weight of water. Distilled water is preferred. The above proportions are not critical and can be departed from if desired. The proportions set forth above have proved highly satisfactory in use.

In applying an aqueous solution or suspension of the novel composition of this invention to hydrophobic tex-

tile fibers, it has been determined, by long experience that the amount of antistatic and lubricating composition carried by a fiber, filament, or yarn lies within a relatively narrow optimum range. Below the range, insufficient lubrication and antistatic properties are obtained while above the range certain properties such as tensile strength and processability are affected adversely. The amount of antistatic and lubricating composition carried by the fibers can be within the range of from about 0.1 percent to 3 percent by weight based on the weight of the fibers. It is preferred, however, that the applied antistatic and lubricating composition be within the relatively narrow range of from about 0.1 percent to 1 percent by weight based on the weight of the fibers.

The following examples are illustrative of this invention. All parts are by weight unless otherwise indicated

#### Example II

Fibers treated in accordance with this example are continuous filament polyester fibers prepared from poly(1,4-cyclohexylenedimethylene terephthalate). Fibers of this type are available commercially under the proprietary designation Kodel. Fibers of this type are well known in the art and can be prepared in accordance with the teachings of Patent 2,901,466.

These fibers, in the form of tow, are treated by spraying with an aqueous emulsion comprised of the following composition:

| Parts |                                                                                                  |
|-------|--------------------------------------------------------------------------------------------------|
| 30    | The monohydroxy oxyethylene oxy 1,2-propylene butyl monoether mixture of Example I ----- 50      |
|       | An approximately equal molar mixture of monolauryl phosphate and dilauryl phosphate ----- 25     |
|       | Morpholine ----- 7                                                                               |
| 35    | Polyoxyethylene glycol having an average molecular weight of about 1540 (Carbowax 1540) ----- 15 |
|       | o-Phenylphenol ----- 3                                                                           |

The treated fibers can be dried in air or they can be placed in an oven maintained at a temperature of from about 105° C. to 110° C. for about an hour to remove from the applied coating substantially all water. In this specific example the fibers are dried in a heated oven. The amount of applied composition is equal to about 0.25 percent by weight based on the weight of the fibers.

The treated tow is satisfactorily processed on a Pacific converter into top. The resulting top is of excellent quality and is substantially free of defects such as clusters and unopened fibers.

#### Example III

Polypropylene staple fibers are treated with an aqueous emulsion of the composition of Example II and in accordance with the procedure described in Example II. The applied composition provides excellent control of static throughout all textile processing operations to which the fibers are subjected. The amount of applied composition in this example is about 0.3 percent by weight of the total weight of the fibers.

#### Example IV

The following composition, in an aqueous medium, is applied by immersion to polyester staple fibers similar to those described in Example II. The amount of applied composition is about 0.25% by weight based on the total weight of the fibers.

| Parts |                                                                                                |
|-------|------------------------------------------------------------------------------------------------|
|       | The monohydroxy oxyethylene oxy 1,2-propylene butyl monoether mixture of Example I ----- 34    |
|       | An approximately equal molar mixture of monolauryl phosphate and dilauryl phosphate ----- 17.5 |
|       | Morpholine ----- 5                                                                             |
| 70    | Polyoxyethylene glycol having an average molecular weight of about 1540 ----- 10.5             |
|       | Polyoxyethylene 200 lauryl amine ----- 30                                                      |
|       | o-Phenylphenol ----- 3                                                                         |

The treated polyester fibers are blended in a 50 percent-50 percent weight ratio with viscose fibers and aged for a week. The test results at the end of this period show excellent antistatic properties of the blend thereby indicating substantially no migration of the applied composition to the hydrophilic viscose fibers. Unblended polyester fibers also show excellent antistatic properties.

*Example V*

Polyester fibers similar to those described in Example II are treated with the following composition in an aqueous medium.

|                                                                                       | Parts   |
|---------------------------------------------------------------------------------------|---------|
| The monohydroxy oxyethylene oxy 1,2-propylene butyl monoether mixture of Example I    | 40 15   |
| An approximately equal molar mixture of mono- lauryl phosphate and dilauryl phosphate | 20      |
| Morpholine                                                                            | 5.6     |
| Polyoxyethylene glycol having an average molecular weight of about 1540               | 12.0 20 |
| N,N-diethylaminoethanol salt of oleyl sulfate                                         | 20      |
| o-Phenylphenol                                                                        | 2.4     |

The amount of the above composition that is applied to the fibers is about 0.25 percent by weight based on the weight of the fibers. The applied lubricant gives excellent control of static and also provides highly satisfactory frictional characteristics for the treated polyester fibers.

Satisfactory results are obtained when either staple fibers or continuous filament fibers are treated with the composition of this invention.

The novel antistatic and lubricating compositions of this invention are adapted particularly for the treatment of synthetic resinous fibers prepared from polyester resins such as polyethylene terephthalate and the polyester resins disclosed in the above examples; polyamide resins such as polycaprolactam (nylon-6), polyhexamethylene adipamide (nylon-66), and polyhexamethylene sebacamide (nylon-68); polyolefins such, for example, as polyethylene, polypropylene and poly-1-butene; and polyacrylates.

Other textile fibers, filaments, yarns and the like that can be treated with the antistatic and lubricating composition of this invention include those prepared from the organic acid esters of cellulose such, for example, as cellulose acetate, cellulose triacetate, cellulose acetate butyrate, and cellulose acetate propionate.

Fibers, filaments, yarns and the like treated with the novel antistatic and lubricating composition of this invention are provided with substantial antistatic protection for prolonged periods of time. A buildup of electrostatic charges on the treated fibers is substantially eliminated.

One of the primary advantages of the novel composition of this invention is that it does not migrate to hydrophilic fibers when hydrophobic fibers, treated with the composition, are blended with or associated with hydrophilic fibers during textile processing steps, thereby providing substantially continued control of static and frictional properties during subsequent textile processing operations.

The compositions of this invention provide for highly satisfactory fiber-to-fiber and fiber-to-metal frictional properties of the treated fibers during processing and the like. They do not corrode textile equipment and have no toxic effects. Furthermore, the novel lubricating and antistatic compositions of this invention when applied to hydrophobic fibers of the type described hereinabove provide treated fibers that have excellent tow opening properties. In addition, the fibers treated with the composition of this invention do not become sticky or gummy on aging and they show excellent heat and light stability.

It is to be understood that the above description and examples are illustrative of this invention and not in limitation thereof.

We claim:

1. Blended fibers having improved antistatic properties, said blend being essentially composed of hydrophilic fibers and polyester staple fibers carrying on said polyester fibers a textile lubricant, said blended fibers being characterized in that after aging for one week the antistatic properties remain substantially unaffected, said lubricant being essentially composed of, by weight,

- (A) from about 20 parts to 75 parts of a water soluble compound which is a mixture of monohydroxy oxyethylene oxy 1,2-propylene aliphatic monoethers having a viscosity of from about 200 to 700 Saybolt Universal Seconds at 100° F. and in which ethylene oxide and 1,2-propylene oxide are combined therein as oxyethylene and oxy 1,2-propylene groups in a weight ratio of 1,2-propylene oxide to ethylene oxide of from 60:40 to 40:60, the monoethers of said mixture containing in a single molecule both the oxyethylene group and the oxy 1,2-propylene group,
- (B) from about 5 parts to 35 parts of a compound selected from the group consisting of monolauryl phosphate, dilauryl phosphate, and mixtures thereof,
- (C) from about 1 part to 10 parts of morpholine,
- (D) from about 5 parts to 25 parts of polyoxyethylene glycol having a molecular weight of from about 1,000 to 2,000, and
- (E) from about 1 part to 5 parts of o-phenylphenol.

2. Blended fibers having improved antistatic properties, said blend being essentially composed of hydrophilic fibers and polyester staple fibers carrying on said polyester fibers a textile lubricant, said blended fibers being characterized in that after aging for one week the antistatic properties remain substantially unaffected, said lubricant being essentially composed of, by weight,

- (A) from about 20 parts to 75 parts of a water soluble compound which is a mixture of monohydroxy oxyethylene oxy 1,2-propylene aliphatic monoethers having a viscosity of from about 200 to 700 Saybolt Universal Seconds at 100° F. and in which ethylene oxide and 1,2-propylene oxide are combined therein as oxyethylene and oxy 1,2-propylene groups in a weight ratio of 1,2-propylene oxide to ethylene oxide of from 60:40 to 40:60, the monoethers of said mixture containing in a single molecule both the oxyethylene group and the oxy 1,2-propylene group,
- (B) from about 5 parts to 35 parts of a compound selected from the group consisting of monolauryl phosphate, dilauryl phosphate, and mixtures thereof,
- (C) from about 1 part to 10 parts of morpholine,
- (D) from about 5 parts to 25 parts of polyoxyethylene glycol having a molecular weight of from about 1,000 to 2,000,
- (E) from about 1 part to 5 parts of o-phenylphenol, and
- (F) polyoxyethylene lauryl amine wherein the polyoxyethylene group has an average molecular weight of about 200 in an amount equal to from about 5% to 30% by weight based on the total weight of (A), (B), (C), (D), and (E).

3. Blended fibers as defined by claim 2 wherein said hydrophilic fibers are viscose fibers and said polyester is poly (1,4-cyclohexylenedimethylene terephthalate).

4. Blended fibers having improved antistatic properties, said blend being essentially composed of hydrophilic fibers and polyester staple fibers carrying on said polyester fibers a textile lubricant, said blended fibers being characterized in that after aging for one week the antistatic properties remain substantially unaffected, said lubricant being essentially composed of, by weight,

- (A) from about 20 parts to 75 parts of a water soluble compound which is a mixture of monohydroxy oxyethylene oxy 1,2-propylene aliphatic monoethers having a viscosity of from about 200 to 700 Saybolt Universal Seconds at 100° F. and in which ethylene oxide and 1,2-propylene oxide are combined therein

as oxyethylene and oxy 1,2-propylene groups in a weight ratio of 1,2-propylene oxide to ethylene oxide of from 60:40 to 40:60, the monoethers of said mixture containing in a single molecule both the oxyethylene group and the oxy 1,2-propylene group, (B) from about 5 parts to 35 parts of a compound selected from the group consisting of monolauryl phosphate, dilauryl phosphate, and mixtures thereof, (C) from about 1 part to 10 parts of morpholine, (D) from about 5 parts to 25 parts of polyoxyethylene glycol having a molecular weight of from about 1,000 to 2,000, (E) from about 1 part to 5 parts of o-phenylphenol, and (F) from about 5% to 25% by weight based on the total weight of (A), (B), (C), (D), and (E) of N,N-diethylaminoethanol salt of oleyl sulfate.

5. Blended fibers having improved antistatic properties, said blend being essentially composed of hydrophilic fibers and polyester staple fibers carrying on said polyester fibers a textile lubricant, said blended fibers being characterized in that after aging for one week the antistatic properties remain substantially unaffected, said lubricant being essentially composed of, by weight,

(A) from about 20 parts to 75 parts of a water soluble compound which is a mixture of monohydroxy oxyethylene oxy 1,2-propylene aliphatic monoethers having a viscosity of from about 200 to 700 Saybolt Universal Seconds at 100° F. and in which ethylene oxide and 1,2-propylene oxide are combined therein as oxyethylene and oxy 1,2-propylene groups in a weight ratio of 1,2-propylene oxide to ethylene oxide of from 60:40 to 40:60, the monoethers of said mixture containing in a single molecule both the

oxyethylene group and the oxy 1,2-propylene group, (B) from about 5 parts to 35 parts of a compound selected from the group consisting of monolauryl phosphate, dilauryl phosphate, and mixtures thereof, (C) from about 1 part to 10 parts of morpholine, (D) from about 5 parts to 25 parts of polyoxyethylene glycol having a molecular weight of from about 1,000 to 2,000, (E) from about 1 part to 5 parts of o-phenylphenol, (F) polyoxyethylene lauryl amine wherein the polyoxyethylene group has an average molecular weight of about 200 in an amount equal to from about 5% to 30% by weight based on the total weight of (A), (B), (C), (D), and (E), and (G) from about 5% to 25% by weight based on the total weight of (A), (B), (C), (D), and (E) of N,N-diethylaminoethanol salt of oleyl sulfate.

#### References Cited by the Examiner

##### UNITED STATES PATENTS

|           |         |                        |            |
|-----------|---------|------------------------|------------|
| 2,278,747 | 4/1942  | Swезеу et al. -----    | 252—8.75   |
| 2,425,755 | 8/1947  | Roberts et al. -----   | 252—8.9 XR |
| 2,597,947 | 5/1952  | Oxley et al. -----     | 252—8.75   |
| 2,614,984 | 10/1952 | Thomas et al. -----    | 252—8.75   |
| 2,690,426 | 9/1954  | Jefferson et al. ----- | 252—8.9 XR |
| 2,743,193 | 4/1956  | Donaldson et al. ----- | 252—8.8 XR |
| 2,803,565 | 8/1957  | Sager -----            | 252—8.9 XR |
| 2,865,855 | 12/1958 | Chandler -----         | 252—8.9    |
| 2,901,466 | 8/1959  | Kibler et al. -----    | 260—75     |
| 3,042,544 | 7/1962  | Marzocchi et al. ----- | 252—8.9 XR |

JULIUS GREENWALD, Primary Examiner.

J. T. FEDIGAN, Assistant Examiner.